# EUROPEAN PATENT SPECIFICATION

(11) **EP 2 512 817 B1**
(45) Date of publication and mention of the grant of the patent: **03.08.2016**
(21) Application number: 09796288.0
(22) Date of filing: 18.12.2009
(51) Int. Cl.: B41N 7/06

(54) **PROCESS FOR MANUFACTURING A METERING ROLL ESPECIALLY USABLE FOR PRINTING AND METERING ROLL OBTAINED BY THIS PROCESS**
VERFAHREN ZUR HERSTELLUNG EINER BESONDERS BEIM DRUCK NÜTZLICHEN DOSIERWALZE UND DURCH DIESES VERFAHREN ERHALTENE DOSIERWALZE
PROCÉDÉ DE FABRICATION D'UN ROULEAU DOSEUR CONVENANT PARTICULIÈREMENT À L'IMPRESSION ET ROULEAU DOSEUR OBTENU AU MOYEN DE CE PROCÉDÉ

(43) Date of publication of application: 24.10.2012
(73) Proprietor: TeroLab Surface Group SA, 1018 Lausanne (CH)
(72) Inventor: LANGER, Gregor, 42781 Haan (DE); DÖRING, Jens-Erich, 41539 Dormagen (DE)
(74) Representative: Nithardt, Roland
(86) International application number: PCT/CH2009/000403
(87) International publication number: WO 2011/072404

(56) References cited:
- WO-A1-91/13762
- GB-A- 2 089 473
- US-A- 3 924 313
- US-A- 5 514 064

## Description

### Technical Field

The present invention concerns a process for manufacturing a metering roll, especially usable in flexographic printing presses, in varnish stations for offset presses and/or in short ink train dry offset presses for example, comprising a central cylindrical core and at least one layer of a hard material peripheral coating.

The present invention concerns also a metering roll, especially usable in flexographic printing presses, in varnish stations for offset presses and/or in short ink train dry offset presses for example, comprising a central cylindrical core and at least one layer of a hard material peripheral coating, obtained by this process.

### Background Art

The metering rolls, are widely used to bring a metered quantity of ink to the plate roll with which it is in contact. One type of metering rolls, is provided with a peripheral coating of ceramic that is engraved, mainly by use of a laser beam. Another type of metering rolls, has a metallic surface layer that is engraved either by mechanical tools or by use of a laser beam. The surface layer is more often made of a soft metal like copper or tin and is chrome plated after the engraving.

Another prior art method consists in a chemical etching of an image that is illuminated by a laser beam or similar.

The United States Patent Nr. 5,514,064 describes a process for making metal inking rolls, particularly for flexographic printing having a roll structure composed of an ammonia hardenable steel, in particular stainless steel.

The UK patent application GB 2 089 473 A relates to an ink doctor roller for printing machines, especially a doctor roller comprising a base body of steel provided with a circumferential covering comprising a sprayed outer layer of wear-resistant material in which a low friction material is embedded in islands.

The international application WO 91/13762 relates to a screen roller comprising a cylindrical roller body and shaft means with a pattern of recesses present on the external surface of the roller body, in which the pattern of recesses is present in an electroplated metal layer which is of a hardness being greater than the hardness of the metal of the roller body.

The technical features which are required for metering rolls, and especially for their superficial coating layer are the following: easiness of the engraving, high resistance to mechanical wear, protection against corrosion due for example to aggressive cleaning products. In particular a ceramic coating is sensitive to corrosive liquids because it is somewhat porous and though it has a great hardness the liquids may penetrate into the coating and reach the lower layers and the central core of the roll. One solution consists in filling up the pores with additional components mixed with the ceramic mixture. When the coating is made of a soft metal, it is necessary to chrome plate the upper layer to harden the surface and increase its resistance.

Furthermore the scraper for metering the printing inks is applied with a high compression on the surface of the upper layer of the metering roll. Due to the hard material of the coating and the sharp edges of the structured surface, the scraper is submitted to an intensive wear.

### Disclosure of Invention

The process of the invention offers a new technology permitting to a manufacture metering roll, having an improved resistance to mechanical wear, a better protection to corrosion at lower costs, and remaining easy to engrave.

Therefore, the process of the present invention such as defined in the preamble is characterized in that the peripheral coating is made of an iron base containing at least one of the elements of the group consisting of chrome, nickel, boron, carbon, molybdenum, silicon, manganese, cobalt and/or at least one of the components of the group consisting of chrome carbide (Cr₃C₂); nickel chrome (NiCr); cobalt chrome (CoCr); tungsten carbide (WC), the peripheral coating being provided by thermal spraying including at least one of the following methods: flame spraying, electrical arc spraying, plasma spraying, high velocity oxy flame spraying or cold gas spraying.

The proportion of chrome is advantageously comprised between 20 and 35%. According to one preferred variant, the proportion of chrome is at least approximately 32%.

According to another preferred variant, the proportion of chrome is at least approximately 27%

The proportion of nickel is advantageously comprised between 0 and 20%.

According to one preferred variant, the proportion of nickel is at least approximately 16%.

According to another preferred variant, the proportion of nickel is at least approximately 8%.

The proportion of boron is advantageously comprised between 0 and 8%. According to one preferred variant the proportion of boron is at least approximately 4.6%.

The proportion of carbon is advantageously comprised between 0 and 3%.

According to one preferred variant the proportion of carbon is at least approximately 0.6%.

According to another preferred variant, the proportion of carbon is at least approximately 2%.

The proportion of molybdenum is advantageously comprised between 0 and 8%.

According to one preferred variant, the proportion of molybdenum is at least approximately 4%.

The proportion of silicon is advantageously comprised between 0 and 2% and preferably between 1 and 3%.

According to one preferred variant, the proportion of silicon is at least approximately 1.2%.

The proportion of manganese is advantageously comprised between 0 and 3%.

According to one variant, the proportion of manganese is at least approximately 0.7%.

The metering roll, of the present invention such as defined in the preamble is characterized in that the peripheral coating is made of an iron base containing at least one of the elements of the group consisting of chrome, nickel, boron, carbon, molybdenum, silicon, manganese, cobalt and/or at least one of the components of the group consisting of chrome carbide (Cr₃C₂); nickel chrome (NiCr); cobalt chrome (CoCr); tungsten carbide (WC), Ni and Co and in that the thickness of this peripheral coating is comprised between 50 and 400 micrometers.

According to one preferred embodiment of the metering roll, the coating is advantageously composed of an iron base with 32% chrome, 8% nickel, 4.6% boron, 0.6% carbon of the total weight.

According to another preferred embodiment of the metering roll, the coating is composed of an iron base with 27% chrome, 16% nickel, 4% molybdenum, 2% carbon, 1.2% silicon, 0.7% manganese of the total weight.

According to a first variant, not forming part of the invention, the coating may be composed of a WC-Ni base containing at least one of the following additional elements: Mo, Cr, C, and the amount of Ni may be at least approximately 8.5%.

When the amount of Ni is at least approximately 8.5%, the amount of Mo is at least approximately 2.2%, the amount of Cr is at least approximately 2.2% and the amount of C is at least approximately 5.7%.

According to a second variant, the coating may be composed of a WC-Fe base containing at least one of the following additional elements: C, Cr, Al, and the amount of Fe may be at least approximately 10.8%.

When the amount of Fe is at least approximately 10.8%, the amount of C is at least approximately 5.6%, the amount of Cr is at least approximately 3.4% and the amount of Al is at least approximately 1%.

### Modes for Carrying Out the Invention

The process of the invention may be used for manufacturing new metering rolls, having a central cylindrical metallic core. The coating is provided by thermal spraying including at least one of the following methods: flame spraying, electrical arc spraying, plasma spraying, high velocity oxy flame spraying or cold gas spraying. After the application of the coating on the surface of the roll, it is first grinded then polished. Afterwards the coating is engraved with a laser beam or by mechanical tools. A further grinding and polishing operation may be necessary for withdrawing remaining protrusions.

It is to be noted that the plasma spraying provides a coating porosity that is higher than the porosity provided by high speed flame spraying

The thickness of the coating is comprised between 50 and 400 micrometers relating to the components that are used and the application planned for the rolls. The resulting corrosion resistance of the coating is higher than 500 hours according the (AASS-test). The hardness of the iron base alloys coating is preferably comprised between 750 and 1000 HV _{0.1}, the hardness of cermets coatings (carbides coatings) is comprised between 800 and 1600 HV _{0.1}. It is to be noted that the hardness of the carbides is much higher than that of the base alloys coatings. However the engraving is harder to do.

According to the invention, the materials that are used to realize the coatings of the rolls may be included in a first group of iron alloys and in a second group of carbides.
Group I : Cr 20-35%; Ni 0-20%; Mo 0-8%; B 0-8%; C 0-3%; Si 0-2%; Mn 0-3%; other elements < 0,1%.
   Variant 1: Preferred composition: Fe Base, Cr 32%, Ni 8%, B 4,6%, C 0,6%.
   Variant 2: Preferred composition: Fe Base, Cr 27%, Ni 16%, C 2%, Si 1,2%, Mn 0,7%.
Group II : Carbide materials (Cermets) WC; Cr₃C₂ in various matrixes with Ni, CoCr and NiCr and Ni or Fe base alloys containing Fe 0-13%; Cr 0-5%; Ni 0-25%; C 0-5%; Mo 0-4%; Al 0-2%; traces < 1%, the rest being WC and/or Cr₃C₂ or alloys.
   Variant 3, not forming part of the invention: WC-Ni-Base (Hastelloy-C) Ni 8,5%; Mo 2,2%; C 5,7% and traces of various elements < 1%.
   Variant 4: WC-Fe base : Fe 10,8%; C 5,6%; Cr 3,4%; Al 1%.

The coatings of variant 1 and variant 2 are preferably applied by means of an atmospheric spraying or by means of a high velocity oxy flame spraying. Gas projection apparatus or liquid projection apparatus may be used for applying the said elements.

Both groups of materials are particularly resistant to mechanical wear and corrosion so that the combination of structured rolls and the scraper will have a higher resistance and a longer working life as a ceramic surface. The coating surface may be structured directly by a laser beam without any further preparation like masking or etching.

## Claims

1. A process for manufacturing a metering roll, especially usable in flexographic printing presses, in varnish stations for offset presses and/or in short ink train dry offset presses for example, comprising a central cylindrical core and at least one layer of a hard material peripheral coating, **characterized in that** the peripheral coating is made of an iron base containing at least one of the elements of the group consisting of chrome, nickel, boron, carbon, molybdenum, silicon, manganese, cobalt and/or at least one of the components of the group consisting of chrome carbide (Cr₃C₂); nickel chrome (NiCr); cobalt chrome (CoCr); tungsten carbide (WC), the peripheral coating being provided by thermal spraying including at least one of the following methods: flame spraying, electrical arc spraying, plasma spraying, high velocity oxy flame spraying or cold gas spraying.

2. A process according to claim 1, **characterized in that** the proportion of chrome is comprised between 20 and 35%.

3. A process according to claim 2, **characterized in that** the proportion of chrome is at least 32%.

4. A process according to claim 2, **characterized in that** the proportion of chrome is at least 27%.

5. A process according to claim 1, **characterized in that** the proportion of nickel is comprised between 0 and 20%.

6. A process according to claim 5, **characterized in that** the proportion of nickel is at least 16%.

7. A process according to claim 5, **characterized in that** the proportion of nickel is at least 8%.

8. A process according to claim 1, **characterized in that** the proportion of boron is comprised between 0 and 8%.

9. A process according to claim 8, **characterized in that** the proportion of boron is at least 4.6%.

10. A process according to claim 1, **characterized in that** the proportion of carbon is comprised between 0 and 3%.

11. A process according to claim 10, **characterized in that** the proportion of carbon is at least 0.6%.

12. A process according to claim 10, **characterized in that** the proportion of carbon is at least 2%.

13. A process according to claim 1, **characterized in that** the proportion of molybdenum is comprised between 0 and 8%.

14. A process according to claim 13, **characterized in that** the proportion of molybdenum is at least 4%.

15. A process according to claim 1, **characterized in that** the proportion of silicon is comprised between 0 and 2% and preferably between 1 and 2%.

16. A process according to claim 15, **characterized in that** the proportion of silicon is at least 1.2%.

17. A process according to claim 1, **characterized in that** the proportion of manganese is comprised between 0 and 3%.

18. A process according to claim 17, **characterized in that** the proportion of manganese is at least 0.7%.

19. A metering roll, especially usable in flexographic printing presses, in varnish stations for offset presses and/or in short ink train dry offset presses for example, obtained by the process according to the preceding claims, said metering roll or similar, usually known as Anilox roll or sleeve, comprising a central cylindrical metallic core and at least one layer of a hard material peripheral coating, **characterized in that** the peripheral coating is made of an iron base containing at least one of the elements of the group consisting of chrome, nickel, boron, carbon, molybdenum, silicon, manganese, cobalt and/or at least one of the components of the group consisting of chrome carbide (Cr₃C₂); nickel chrome (NiCr); cobalt chrome (CoCr); tungsten carbide (WC), and **in that** the thickness of the coating is comprised between 50 and 400 micrometers.

20. A metering roll, according to claim 19, **characterized in that** the peripheral coating is composed of an iron base with 32% chrome, 8% nickel, 4.6% boron, 0.6% carbon of the total weight.

21. A metering roll, according to claim 19, **characterized in that** the peripheral coating is composed of an iron base with 27% chrome, 16% nickel, 4% molybdenum, 2% carbon, 1.2% silicon, 0.7% manganese of the total weight.

22. A metering roll, according to claim 19, **characterized in that** the peripheral coating contains at least one of the following additional elements: Mo, Cr, C, Ni.

23. A metering roll, according to claim 19, **characterized in that** the peripheral coating is composed of a WC-Fe base containing at least one of the following additional elements: C, Cr, Al.

24. A metering roll, according to claim 23, **characterized in that** the amount of Fe is at least 10.8%.

25. A metering roll, according to claim 23, **characterized in that** the amount of Fe is at least 10.8%, the amount of C is at least 5.6%, the amount of Cr is at least 3.4% and the amount of Al is at least 1 %.

## Patentansprüche

1. Verfahren zur Herstellung einer Dosierwalze, die zum Beispiel insbesondere bei flexographischen Druckerpressen, bei Lackierstationen für Offsetpressen und/oder bei Kurzfarbwerktrocken-Offsetpressen verwendbar ist, die einen mittleren, zylindrischen Kern und wenigstens eine Schicht aus einer Umfangsbeschichtung aus einem harten Material aufweist,
**dadurch gekennzeichnet, dass**
die Umfangsbeschichtung aus einer Eisenbasis hergestellt wird, die wenigstens eines der Elemente aus der Gruppe aufweist, die aus Chrom, Nickel, Bor, Karbon, Molybdän, Silizium, Mangan, Kobalt besteht und/oder wenigstens eine der Komponenten aus der Gruppe aufweist, die aus Chromkarbid (Cr₃C₂); Nickelchrom (NiCr); Kobaltchrom (CoCr); Wolframkarbid (WC) besteht, wobei die Umfangsbeschichtung durch thermisches Sprühen einschließlich wenigstens eines der folgenden Verfahren erzeugt wird: Flammsprühen, elektrisches Bogensprühen, Plasmasprühen, Hochgeschwindigkeits-Oxiflammsprühen oder Kaltgassprühen.

2. Verfahren nach Anspruch 1,
**dadurch gekennzeichnet, dass**
der Anteil von Chrom zwischen 20 und 35 % enthalten ist.

3. Verfahren nach Anspruch 2,
**dadurch gekennzeichnet, dass**
der Anteil von Chrom wenigstens 32 % beträgt.

4. Verfahren nach Anspruch 2,
**dadurch gekennzeichnet, dass**
der Anteil von Chrom wenigstens 27 % beträgt.

5. Verfahren nach Anspruch 1,
**dadurch gekennzeichnet, dass**
der Anteil von Nickel zwischen 0 und 20 % enthalten ist.

6. Verfahren nach Anspruch 5,
**dadurch gekennzeichnet, dass**
der Anteil von Nickel wenigstens 16 % beträgt.

7. Verfahren nach Anspruch 5,
**dadurch gekennzeichnet, dass**
der Anteil von Nickel wenigstens 8 % beträgt.

8. Verfahren nach Anspruch 1,
**dadurch gekennzeichnet, dass**
der Anteil von Bor zwischen 0 und 8 % enthalten ist.

9. Verfahren nach Anspruch 8,
**dadurch gekennzeichnet, dass**
der Anteil von Bor wenigstens 4,6 % beträgt.

10. Verfahren nach Anspruch 1,
**dadurch gekennzeichnet, dass**
der Anteil von Kohlenstoff zwischen 0 und 3 % enthalten ist.

11. Verfahren nach Anspruch 10,
**dadurch gekennzeichnet, dass**
der Anteil von Kohlenstoff wenigstens 0,6 % beträgt.

12. Verfahren nach Anspruch 10,
**dadurch gekennzeichnet, dass**
der Anteil von Kohlenstoff wenigstens 2 % beträgt

13. Verfahren nach Anspruch 1,
**dadurch gekennzeichnet, dass**
der Anteil von Molybdän zwischen 0 und 8 % enthalten ist.

14. Verfahren nach Anspruch 13,
**dadurch gekennzeichnet, dass**
der Anteil von Molybdän wenigstens 4 % beträgt.

15. Verfahren nach Anspruch 1,
**dadurch gekennzeichnet, dass**
der Anteil von Silizium zwischen 0 und 2 % und vorzugsweise zwischen 1 und 2 % enthalten ist.

16. Verfahren nach Anspruch 15,
**dadurch gekennzeichnet, dass**
der Anteil von Silizium wenigstens 1,2 % beträgt.

17. Verfahren nach Anspruch 1,
**dadurch gekennzeichnet, dass**
der Anteil von Mangan zwischen 0 und 3 % enthalten ist.

18. Verfahren nach Anspruch 17,
**dadurch gekennzeichnet, dass**
der Anteil von Mangan wenigstens 0,7 % beträgt.

19. Dosierwalze, die zum Beispiel insbesondere bei flexographischen Druckerpressen, bei Lackierstationen für Offsetpressen und/oder bei Kurzfarbwerktrocken-Offsetpressen verwendbar ist, erhalten durch den Prozess nach einem der vorhergehenden Ansprüche, wobei die Dosierwalze oder ähnliches, üblicherweise als Anilox-Walze oder -buchse bekannt, einen mittleren, zylindrischen, metallischen Kern und wenigstens eine Schicht aus einer Umfangsbeschichtung aus einem harten Material aufweist,
**dadurch gekennzeichnet, dass**
die Umfangsbeschichtung aus einer Eisenbasis hergestellt ist, die wenigstens eines der Elemente aus der Gruppe aufweist, die aus Chrom, Nickel, Bor, Karbon, Molybdän, Silizium, Mangan, Kobalt besteht und/oder wenigstens eine der Komponenten aus der Gruppe aufweist, die aus Chromkarbid (Cr₃C₂); Nickelchrom (NiCr); Kobaltchrom (CoCr); Wolframkarbid (WC) besteht, und dass die Dicke der Beschichtung zwischen 50 und 400 Mikrometer beträgt.

20. Dosierwalze nach Anspruch 19,
**dadurch gekennzeichnet, dass**
die Umfangsbeschichtung aus einer Eisenbasis mit 32 % Chrom, 8 % Nickel, 4,6 % Bor, 0,6 % Kohlenstoff des Gesamtgewichts zusammengesetzt ist.

21. Dosierwalze nach Anspruch 19,
**dadurch gekennzeichnet, dass**
die Umfangsbeschichtung aus einer Eisenbasis mit 27 % Chrom, 16 % Nickel, 4 % Molybdän, 2 % Kohlenstoff, 1,2 % Silizium, 0,7 % Mangan des Gesamtgewichts zusammengesetzt ist.

22. Dosierwalze nach Anspruch 19,
**dadurch gekennzeichnet, dass**
die Umfangsbeschichtung wenigstens eines der folgenden zusätzlichen Elemente aufweist: Mo, Cr, C, Ni.

23. Dosierwalze nach Anspruch 19,
**dadurch gekennzeichnet, dass**
die Umgangsbeschichtung aus einer WC-Fe-Basis zusammengesetzt ist, die wenigstens eines der folgenden zusätzlichen Elemente aufweist: C, Cr, Al.

24. Dosierwalze nach Anspruch 23,
**dadurch gekennzeichnet, dass**
die Menge von Fe wenigstens 10,8 % beträgt.

25. Dosierwalze nach Anspruch 23,
**dadurch gekennzeichnet, dass**
die Menge von Fe wenigstens 10,8 % beträgt, die Menge von C wenigstens 5,6 % beträgt, die Menge von Cr wenigstens 3,4 % beträgt und die Menge von Al wenigstens 1 % beträgt.

## Revendications

1. Procédé de fabrication d'un rouleau d'impression, en particulier utilisable dans les procédés d'impression par flexographie, dans des stations de coloration pour presses offset et/ou dans des presses offset à encres sèches par exemple, comportant un noyau cylindrique central et au moins une couche périphérique d'un revêtement en un matériau dur, **caractérisé en ce que** le revêtement périphérique est réalisé avec une base en acier contenant au moins un des éléments du groupe composé de chrome, nickel, bore, carbone, molybdène, silicium, manganèse, cobalt et/ou au moins un des composants du groupe composé de carbure de chrome (Cr₃C₂); de chrome nickel (NiCr); de chrome cobalt (CoCr); de carbure de tungstène (WC), le revêtement périphérique étant effectué par une pulvérisation thermique comprenant au moins l'une des méthodes suivantes :pulvérisation à la flamme, pulvérisation par arc électrique, pulvérisation par plasma, pulvérisation à la flamme à oxygène à grande vitesse, ou pulvérisation au gaz froid.

2. Procédé selon la revendication 1, **caractérisé en ce que** la proportion de chrome est comprise entre 20 and 35%.

3. Procédé selon la revendication 2, **caractérisé en ce que** la proportion de chrome est au moins de 32%.

4. Procédé selon la revendication 2, **caractérisé en ce que** la proportion de chrome est au moins de 27%.

5. Procédé selon la revendication 1, **caractérisé en ce que** la proportion de nickel est comprise entre 0 et 20%.

6. Procédé selon la revendication 5, **caractérisé en ce que** la proportion de nickel est au moins de 16%.

7. Procédé selon la revendication 5, **caractérisé en ce que** la proportion de nickel est au moins de 8%.

8. Procédé selon la revendication 1, **caractérisé en ce que** la proportion de bore est comprise entre 0 et 8%.

9. Procédé selon la revendication 8, **caractérisé en ce que** la proportion de bore est au moins de 4,6%,

10. Procédé selon la revendication 1, **caractérisé en ce que** la proportion de carbone est comprise entre 0 et 3%.

11. Procédé selon la revendication 10, **caractérisé en ce que** la proportion de carbone est au moins de 0.6%.

12. Procédé selon la revendication 10, **caractérisé en ce que** la proportion de carbone est au moins de 2%.

13. Procédé selon la revendication 1, **caractérisé en ce que** la proportion de molybdène est comprise entre 0 et 8%.

14. Procédé selon la revendication 13, **caractérisé en ce que** la proportion de molybdène est au moins de 4%.

15. Procédé selon la revendication 1, **caractérisé en ce que** la proportion de silicium est comprise entre 0 et 2% et de préférence entre 1 et 2%.

16. Procédé selon la revendication 15, **caractérisé en ce que** la proportion de silicium est au moins de 1,2 %.

17. Procédé selon la revendication 1, **caractérisé en ce que** la proportion de manganèse est comprise entre 0 et 3%.

18. Procédé selon la revendication 17, **caractérisé en ce que** la proportion de manganèse est au moins de 0.7%.

19. Rouleau d'impression, en particulier utilisable dans les procédés d'impression par flexographie, dans des stations de coloration pour presses offset et/ou dans des presses offset à encres sèches par exemple, obtenu par le procédé selon les revendications précédentes, ledit rouleau d'impression ou similaires, habituellement connu comme rouleau ou manchon Anilox, comportant un noyau cylindrique central et au moins une couche périphérique d'un revêtement en un matériau dur, **caractérisé en ce que** le revêtement périphérique est réalisé avec une base en acier contenant au moins un des éléments du groupe composé de chrome, nickel, bore, carbone, molybdène, silicium, manganèse, cobalt et/ou au moins un des composants du groupe composé de carbure de chrome (Cr₃C₂); de chrome nickel (NiCr); de chrome cobalt (CoCr); de carbure de tungstène (WC), et **en ce que** l'épaisseur du revêtement est comprise entre 50 and 400 micromètres.

20. Rouleau d'impression selon la revendication 19, **caractérisé en ce que** le revêtement périphérique est réalisé en une base en acier contenant 32% de chrome, 8% de nickel, 4,6% de bore, 0,6% de carbone du poids total.

21. Rouleau d'impression selon la revendication 19, **caractérisé en ce que** le revêtement périphérique est réalisé en une base en acier contenant 27% de chrome, 16% de nickel, 4% de molybdène, 2% de carbone, 1,2% de silicium, 0,7% de manganèse du poids total.

22. Rouleau d'impression selon la revendication 19, **caractérisé en ce que** le revêtement périphérique contient au moins l'un des éléments additionnels suivants : Mo, Cr, C, Ni.

23. Rouleau d'impression selon la revendication 19, **caractérisé en ce que** le revêtement périphérique est réalisé en une base en WC-Fe contenant au moins l'un des éléments additionnels suivants : C, Cr, Al.

24. Rouleau d'impression selon la revendication 23, **caractérisé en ce que** la quantité de Fe est au moins de 10.8%.

25. Rouleau d'impression selon la revendication 23, **caractérisé en ce que** la quantité de Fe est au moins de 10.8%, la quantité de C est au moins de 5.6%, la quantité de Cr est au moins de 3.4% et la quantité de Al est au moins de 1%.
